

# UNITED STATES PATENT OFFICE.

HACHIG M. BULUCKIAN, OF CLEVELAND, OHIO.

## PROCESS FOR HARDENING ALUMINUM.

1,336,420.

Specification of Letters Patent. Patented Apr. 13, 1920.

No Drawing.

Application filed May 31, 1919. Serial No. 301,083.

To all whom it may concern:

Be it known that I, HACHIG M. BULUCKIAN, a citizen of Armenia, having declared my intention to become a citizen of the 5 United States of America, residing at Cleveland, in the county of Cuyahoga and State of Ohio, have invented certain new and useful Improvements in Processes for Hardening Aluminum, of which the following 10 is a specification.

Aluminum (Al) of commerce is a rather soft white metal of low specific gravity melting at 655° C. and because of its exceedingly low specific gravity, the same is 15 especially serviceable where lightness in weight is a requisite, such as aeroplane use as well as boats, automobiles, and many other articles, the metal being capable of a high polish. The softness of aluminum and 20 its weakness in standing strains, has long been a drawback in preventing such use as the sacrifice of strength for lightness is impossible in construction work.

The primary object of my invention 25 therefore, is the provision of a process for treating aluminum, whereby the pure aluminum of commerce testing approximately 99.9% pure and at about (scleroscope test) 4 for hardness is increased in hardness to test 30 at nearly 12 without the addition of alloying metals. The production of aluminum alloys increases the weight of pure aluminum proportional to the amount of the alloy which is added while my invention increases the hardness of aluminum 300% no 35 addition is made to the weight, no metal alloys are used, nor chemicals as such employed.

This being the general object of my invention, the same will now be fully described, using as a manner of illustration one formula employed for increasing the hardness of aluminum from 4 to 12 under scientific tests, it being understood that minor 45 changes may be made in the described process in the exact proportion of the ingredients or the use of equivalents without departing from the spirit and scope of my invention as claimed.

50 First, pure commercial aluminum is melted and thereto is added substantially 1/34th by bulk of gum-glutin preferably in

powdered form and having great adhesive strength. This gum-glutin is the roots of numerous plants of the *Acacia* family 55 mostly native in Egypt, Armenia, and Turkey, where the same is very cheap but also found to a slight extent in America, where it is higher in price. The acacia roots are ground or powdered into meal or flour 60 and a small quantity of the powder is added to the batch of molten aluminum producing a bubbling whereby the gum-glutin affects the entire mass. In a quantity of 8 ounces melted aluminum the admixture of 1/8th 65 ounce acacia root flour is practicable. Gum-glutin may be also advantageously employed in powdered form produced from roots of other plants and vegetation native in Egypt, Armenia and Turkey such as 70 reeds and rushes.

Second, a small flake of oyster shell is added to the molten batch, the amount necessary for the 8 ounces of aluminum above noted, being a thin flake 1/4th inch in 75 diameter of any variety of oyster shell. This addition causes the mass to bubble throughout, so that the properties of the oyster shell affects the entire quantity.

Third, gum arabic is added to the batch in 80 a quantity substantially twice the size of the oyster shell and this becomes mixed with the entire batch.

Upon completion of such mixture, the batch is allowed to cool and upon reaching 85 the temperature of the atmosphere, the aluminum will be substantially three times the hardness of the pure aluminum being treated. Only the elements herein stated have been added to the pure aluminum and in 90 small quantities not detracting from the purity of the metal which remains unalloyed with its original purity upon completion of the process possessing a testing strength of 12.

95 The sequence of the steps may be changed at will, as to the addition of gum-glutin powder, oyster shell, and gum-arabic to the melted pure aluminum. The pure aluminum so treated by the preferred form of my 100 process, loses none of its original properties, of lightness in weight, capacity for finish, not readily oxidized by air, nor corroded by organic acids.

Having thus described my invention what I claim as new and desire to secure by Letters Patent is:—

1. A process for hardening aluminum consisting in adding gum-glutin, oyster shell and gum arabic to molten pure aluminum.
2. A process of the character described,

consisting in melting aluminum, adding thereto substantially 1/64th of the quantity of flour produced from gum-glutin plant roots and a flake of oyster shell and a quantity of gum arabic substantially double the size of the shell flake.

In testimony whereof I affix my signature. 15

HACHIG M. BULUCKIAN.